

April 25, 1939.

G. B. JONAS

2,156,019

PERMANENT MAGNET STEEL ALLOY AND METHOD OF MAKING SAME

Filed Feb. 10, 1936



Fig. 1

Fig. 2



Fig. 3

INVENTOR  
GOTTFRIED BRUNO JONAS

BY

*G. B. Jonas*  
ATTORNEY.

## UNITED STATES PATENT OFFICE

2,156,019

PERMANENT MAGNET STEEL ALLOY AND  
METHOD OF MAKING SAMEGottfried Bruno Jonas, Eindhoven, Netherlands,  
assignor to N. V. Philips' Gloeilampenfabrieken,  
Eindhoven, NetherlandsApplication February 10, 1936, Serial No. 63,236  
In Germany March 5, 1935

2 Claims. (Cl. 175—21)

My invention relates to alloy steels for permanent magnets and more particularly to alloy steels containing nickel and aluminium.

It has been proposed, for instance in the U. S. Patent #2,027,994 to Mishima, to make permanent magnets from an Al-Ni-Fe alloy without quenching or annealing. Although this elimination of special heat treatment simplified and reduced the cost of manufacture, I have found that for alloys containing 15 to 25% Ni and 7% to 15% Al, the resulting magnets had poor magnetic properties unless they were subjected to special heat treatments.

The object of my invention is to improve the magnetic properties of such alloys without the use of special heat treatment, and for this purpose I add to the alloy between about 0.5 to 5% Ti, the actual quantity of Ti being dependent upon the dimensions of the casting.

In order that the invention can be clearly understood and readily carried into effect, I shall describe the same in more detail in comparison with the prior art and with reference to the accompanying drawing, in which Figures 1 to 3 are graphs giving the magnetic curves of permanent magnets according to the invention.

It is known to make permanent magnets from steel alloys containing nickel and aluminium, such steels being described for instance, in the French Patent No. 731,361, as well as in an article by Kotaro Honda in the periodical "Metallwirtschaft, Wissenschaft und Technik" (Number 24 of June 15, 1934). The magnet steels described in the French patent are made from iron to which from about 5% to 40% of nickel and from 1 to 20% of aluminium are added, with the possible addition of cobalt, manganese, tungsten, molybdenum, vanadium or copper.

The French patent states that such nickel-aluminium steels have very favourable magnetic properties without being hardened, and thus have the advantage of being usable in their cast state without requiring any hardening by thermal treatment. Furthermore, from the figures given regarding the magnetic properties of these alloys it would appear that this patent gives the remanence of all of these Al-Ni steels as exceeding 9,000 gauss, whereas all of the maximum values of their coercive force exceeds 400 gauss.

However, in practice it has been found that for the steels of such composition, such high values could not be even approximated without hardening, and even with the aid of a heat treatment these values could not be obtained. Extensive tests have conclusively proven that the statement that such Ni-Al alloys have such excellent magnetic properties in their cast state, without subsequent heat treatment, is erroneous.

in all cases, or at least in the greater number of possible cases.

The patent neglects the fact that for a casting made of a steel of a definite composition, the size of the casting as well as the thermal properties of the mould are of great importance with respect to the resulting magnetic properties of the steel because the cooling speed has a determinative influence on same.

I have found that when making magnets of 10 the size used for example for magnets of dynamic speakers, from such Al-Ni alloy steels without hardening, the magnetic properties thereof are as a rule inferior to those made of the well-known cobalt steels and that only when 15 subjected to a definite thermal treatment, do the Ni-Fe-Al alloys show marked superiority over cobalt steels.

The above will be illustrated by a series of tests, made on test pieces of Ni-Fe-Al alloys 20 having a length of 33 mm., a width of 27 mm. and a thickness of 10 mm.; these pieces having been cut from cast bars of a length of 150 mm., a width of 27 mm. and a thickness of 10 mm. The dimensions of the test pieces are even more 25 favorable for reaching high magnetic values than are the dimensions of most magnets used in practice.

## Test I

This test was made on a piece of the above 30 size having a composition of 25% nickel, 11% aluminium, and the remainder iron. In its cast state and without thermal treatment, this piece had a remanence of 5200 gauss and a coercive 35 force of 325 gauss. After being subjected to thermal treatment by hardening from a temperature of 1200° C. in an oil bath at room temperature, and subsequent annealing at a temperature of from 650° C. to 750° C., the test piece had a 40 remanence of 7200 gauss and a coercive force 45 of 400 gauss.

## Test II

A test piece of the above size and having a 45 composition of 27% nickel, 12% aluminium and the remainder iron, in its cast state had a remanence of 4400 gauss and a coercive force of 400 gauss. After the test piece was thermally treated in the same manner as given in Test I, 50 it had a remanence of 7000 gauss and a coercive force of 490 gauss.

## Test III

A test piece of the above size and having a composition of 30% nickel, 14% aluminium and the remainder iron, in its cast state and without thermal treatment, had a remanence of 3600 gauss and a coercive force of 450 gauss. After being subjected to the same thermal treatment as given in Test I, this piece had a remanence of

5600 gauss and a coercive force of 620 gauss. Even if in certain special individual cases which seldom occur in practice, for instance when using very thin-walled castings, mould materials of a very high thermal conductivity, etc. higher values are obtained without thermal treatment, it appears that the magnetic values given in the French specification cannot be obtained without a special heat treatment. In 10 any case, the French patent does not teach one skilled in the art how to obtain any appreciable advantage by using the Al-Ni-Fe steels.

The object of my invention is to provide a magnet steel alloy which is much less sensitive 15 to the cooling speed and which, in its cast state, has much better magnetic properties than the castings cast under normal conditions from the alloys described in the French patent. Furthermore, castings of the alloy according to the invention without being heat-treated have magnetic properties which closely approximate the magnetic properties of hardened castings made from the alloy of the French patent.

According to the invention, I add to an alloy 25 containing iron as a base material, and in addition about 15% to 25% nickel and about 7% to 15% aluminium, a quantity of titanium—usually from 5% to 5%—which depends on the size of the magnet to be manufactured, and which 30 should be substantially exactly in the amount required to make quenching of the casting unnecessary. With such an alloy good magnets can be produced from the ordinary sand castings without any further heat treatment, provided their size is not too large.

According to the invention, magnets having very good magnetic properties can be produced from alloys having the following composition:

|                | Percent   |
|----------------|-----------|
| 40 Nickel..... | 22        |
| Aluminium..... | 11        |
| Titanium.....  | 3         |
| Iron.....      | Remainder |

Magnets made from alloys of the above composition have a remanence of about 6400 gauss and a coercive force of about 500 gauss; for magnet sizes having a ratio between their surface area in sq. mms. and their volume in cu. mms. of about 1 to 3½. The size of the magnet is specified because the remanence and coercive force are dependent thereon, and if the above ratio between the surface area and volume is changed, the values of remanence and coercive force will also change to some extent.

The magnetic properties of magnets made according to the invention are indicated in the accompanying drawing, in which Figures 1 to 3 are magnetization curves.

The results which can in practice be obtained by the present invention will be better understood by giving the following example from loudspeaker practice. Magnet rings for moving coil loudspeakers, for instance, were made which were given the following dimensions:

|                        | Millimeters |
|------------------------|-------------|
| External diameter..... | 72          |
| Internal diameter..... | 49          |
| Height.....            | 22          |

70 Ratio of surface area in sq. cms. to volume in cu. cms. equals 1 to 2.7. Such a magnet was obtained by fusing together 27% Ni, 12.5% Al, the remainder being iron, at a casting temperature of at least about 1450° C. cast in sand, cooling 75 down in the sand mould and subsequent mag-

netisation and gave the following magnetic values:

|                        |      |
|------------------------|------|
| Remanence Br.....      | 3400 |
| Coercive force Hc..... | 390  |

After a suitable heat treatment (quenching from a temperature of 1200–1300° C. in an oil bath to room temperature, and subsequently annealing for about half an hour at about 675° C.) and subsequent magnetisation the following 10 values were obtained:

|         |      |
|---------|------|
| Br..... | 6000 |
| Hc..... | 540  |

The same magnet cast in the composition 15 stated by the invention and in which, in contradistinction to the last-mentioned composition of 27% Ni, part of the Ni is replaced by titanium, in this case 22% Ni, 11% Al, 3% Ti (from 12% ferro-titanium), the remainder being iron, at a 20 casting temperature of at least about 1450° C. cast in sand, after cooling in the sand mould and subsequent magnetisation gave:

|         |      |
|---------|------|
| Br..... | 6150 |
| Hc..... | 540  |

Thus it appears from the last-mentioned example of the invention that without using a special heat treatment, magnetic values at Br 6150, Hc 540 can be obtained. These are of practical use in loudspeaker construction, and are furthermore of the same order of magnitude as those values (Br:6000, Hc 540), which according to the previously stated example, are obtained only by heat treatment.

In the Figures 1 to 3 the abscissae represent 35 coercive force in gauss and the ordinates represent remanence in gauss.

Referring to Figure 1, the magnetization 40 curves 1, 2, 3 and 4 represent the test results obtained on four pieces, all of the pieces being in their cast state without heat treatment. The difference found between the four curves is principally due to the fact that the constituents of the alloy were added in different order and to some extent in different forms when making the 45 castings for the test pieces.

For instance, titanium is added in its pure state, but preferably it forms a constituent of a commercial ferro-alloy which may have the following composition:

|         | Percent |
|---------|---------|
| Fe..... | 59.4    |
| Ti..... | 26.2    |
| Si..... | 1.4     |
| C.....  | 0.0067  |
| Cu..... | 3.00    |
| Al..... | 10.0    |

The use of titanium in this form is preferable 60 because it is cheaper than using titanium in its pure state.

It has been found that the other constituents of the mentioned ferro-titanium alloy are not of great importance for the magnetic properties of the magnetic alloy. The improved results obtained by using the ferro-titanium alloy instead of pure titanium are probably due to the fact that smaller consumption losses occur during the alloying and thus the desired composition of the magnetic alloy can be more accurately obtained. 70 Furthermore, it has been found advantageous to add the aluminium last, because somewhat improved magnetic properties may be obtained in this way.

From curves 1 to 4 of Figure 1 it will be noted 75

that the remanences of the test pieces range between about 5700 and 6400, whereas the coercive forces range between about 420 and 520.

The curves 1', 2', 3' and 4' of Fig. 2 were obtained with the test pieces, which without heat-treatment gave curves 1, 2, 3, and 4 respectively, after these test pieces had been annealed for one hour at a temperature of between 650 to 675° C. Comparison of the curves of Figs. 1 and 2 shows practically no difference in the magnetic properties of the test pieces before and after their annealing.

That annealing has practically no effect more clearly appears from Fig. 3 in which curve A represents the average of curves 1, 2, 3, and 4 of Fig. 1, whereas curve B represents the average of curves 1', 2', 3', and 4' of Fig. 2. Comparison of curves A and B shows that the annealing of the test pieces has no appreciable effect upon either the coercive force or the magnitude  $B \times H_{max}$ . Furthermore, annealing only slightly increases the remanence of the test pieces above that of the cast pieces before heat treatment.

The Ni-Al-Ti-Fe alloys should not be subjected at all to the normal hardening operation, as this greatly deteriorates their magnetic properties. For instance, when the test piece corresponding to curves 1 and 1' was subjected to a hardening and an annealing process, (quenching in oil or water, from 1150-1300° C. to room temperature and annealing to about 650-675° C.) its remanence was reduced to about 5000 gauss, and its coercive force reduced to about 300 gauss. Normal hardening of the magnets

is, as a rule, also impossible as it usually results in fracture or cracking of same.

Reduction of the average titanium content slightly increases the remanence but reduces the coercive force to such an extent as to produce a steel of inferior magnetic properties. Also too small a titanium content renders the alloy more sensitive to thermal treatment. On the other hand, increasing the titanium content above 3% is objectionable, in that it renders the casting 10 so brittle as to cause a certain percentage of waste by breakage.

Zirconium and antimonium have similar effect to titanium and can replace partly the titanium as such addition. However, as their effect is usually less than that of the titanium, I prefer as a rule, to use titanium.

While I have described my invention in connection with specific examples, and in specific applications, I do not wish to be limited thereto, but desire the appended claims to be construed as broadly as permissible in view of the prior art.

What I claim is:

1. An unquenched cast permanent magnet consisting substantially of 22% Ni, 11% Al, 3% Ti, and the remainder substantially Fe.
2. A method of making a permanent magnet casting comprising forming an alloy consisting substantially of 22% Ni, 11% Al, 3% Ti, and the remainder substantially iron, casting the alloy in a mold, and heat-treating the casting solely by slowly cooling the same in the mold.

GOTTFRIED BRUNO JONAS.